

# United States Patent

Göthel et al.

[15] 3,674,692

[45] July 4, 1972

[54] **LUBRICANTS AND POWER  
TRANSMISSION FLUIDS ON THE BASIS  
OF CARBOXYLIC ACID ESTERS**

[72] Inventors: **Herbert Göthel, Oberhausen-Holten; Hans Feichtinger, Dinslaken, both of Germany**

[73] Assignee: **Ruhrchemie AG, Oberhausen-Holten, Germany**

[22] Filed: **May 13, 1970**

[21] Appl. No.: **37,043**

[30] **Foreign Application Priority Data**

May 16, 1969 Germany .....P 19 25 048.7

[52] U.S. Cl. ....**252/56 S, 252/79, 260/485 R**

[51] Int. Cl. ....**C10m 1/26**

[58] **Field of Search** .....**252/565, 79**

[56]

**References Cited**

**UNITED STATES PATENTS**

|           |        |                        |            |
|-----------|--------|------------------------|------------|
| 3,309,318 | 3/1967 | Aylesworth et al. .... | 252/56 S   |
| 2,548,493 | 4/1951 | Robey. ....            | 252/56 S X |
| 3,048,542 | 8/1962 | Tierney et al. ....    | 252/56 S X |

*Primary Examiner*—Daniel E. Wyman

*Assistant Examiner*—W. Cannon

*Attorney*—Burgess, Dinklage & Sprung

[57]

**ABSTRACT**

A MIL 7808 lubricant and power transmission fluid comprising:

55 to 70 weight percent hexane-1, 6-diol-isononanoate-ethylhexanoate;

15 to 30 weight percent 2,2-dimethylpropanediol-pelargonate-nonanoate; and

10 to 20 weight percent octyl-nonyl-trimethyladipate.

**3 Claims, No Drawings**

## LUBRICANTS AND POWER TRANSMISSION FLUIDS ON THE BASIS OF CARBOXYLIC ACID ESTERS

Lubricating oils, especially those intended for use in subsonic jet propulsion aircraft engines as well as power transmission fluids for use under extreme temperature conditions, must meet certain demands which are summarized for instance in USA Military Specification MIL-L-007808 F (so-called 7808 fluids). Oils corresponding to this standard specification must possess the following properties: viscosities above 3 cSt at 98.9°C and below 13,000 cSt at -53.9°C; flame points above 204°C; and setting points below -60°C. Furthermore they must meet certain demands with respect to corrosion as well as oxidation stability, which are likewise standardized.

Heretofore, esters of sebacic acid were generally used for this purpose (see Gunderson and Hart, Synthetic lubricants, New York, 1962, chapter 5 "Dibasic acid esters").

Owing to the increasing requirements in high-grade lubricants and power transmission fluids, it is an object of the invention to provide ester-oils for use as lubricants, especially for turbine engines, as well as for power transmission fluids, which can economically be prepared in simple manner from easily obtainable, commercially available alcohol and acid components, which meet the hereinbefore-mentioned demands, particularly the 7808 specifications.

In accordance with the present invention it has now been found that these objects may be accomplished by lubricants and power transmission fluids, comprising 55 to 70 percent by weight hexane-1,6-diol-isobornanoate-ethylhexanoate, 15 to 30 percent by weight 2,2-dimethylpropanediol-pelargonate-nonoanoate and 10 to 20 percent by weight octyl-nonyl-trimethyladipate.

Oils of the following composition possess especially valuable properties and are preferred: 60 to 65 percent by weight hexane-1,6-diol-isobornanoate-ethylhexanoate, 20 to 24 percent by weight 2,2-dimethylpropanediol-pelargonate-nonoanoate and 13 to 17 percent by weight octyl-nonyl-trimethyladipate.

Each of these esters is derived from three different components. The esters derived from glycols are prepared by reaction thereof with two different monocarboxylic acids as specified. The ester of trimethyladipic acid is obtained by reaction of this acid with the two different mono-alcohol components. The esterification may be performed by any esterification process known in the art and is per se conventional.

In the hexane-1,6-diol-isobornanoate-ethylhexanoate, the acids should have a moiety mole ratio to each other, respectively, of about 0.9 to 1.1, preferably about equimolar proportions.

In the 2,2-dimethylpropanediol-pelargonate-nonoanoate, the acids should have a moiety mole ratio to each other, respectively, of about 0.9 to 1.1, preferably about equimolar proportions.

In the octyl-nonyl-trimethyladipate, the alcohols have a moiety mole ratio to each other, respectively, of about 0.9 to 1.1, preferably about equimolar proportions.

The ester oil composition according to the invention is prepared by simple admixture of the esters in the appropriate specified quantities and including conventional additives as, for instance, oxidation inhibiting compounds or antifoaming agents as may be required or desired.

None of the individual components of the composition of this invention complies with the hereinbefore-mentioned requirements, as can be seen from the following. The ester 2,2-dimethylpropane-1,3-diol-isobornanoate-pelargonate for instance, which, owing to its quaternary carbon atom, is heat and oxidation resistant, possesses a viscosity of 10,200 cSt at -53.9°C, a setting point of -70°C, and a flame point of 208°C, but its viscosity of 2.94 cSt at 98.9°C ranges below the standard value of 3 cSt. The ester n-Oxo-octyl-n-Oxo-nonyl-trimethyladipate, which, due to its structure, also exhibits thermal and oxidation stability, meets the said demands with a viscosity of 3.2 cSt at 98.9°C, a flame point of 229°C and a

setting point of -69.0°C but its viscosity of 17,100 cSt at -53.9°C is higher than the standard value of 13,000 cSt. Hexane-1,6-diol-isobornanoate-ethylhexanoate satisfies the requirements of viscosity of 3.17 cSt at 98.9°C, of 11,800 at -53.9°C; of setting point of -70°C and of flame point of 217°C, but its heat and oxidation stability is less than that of the two other esters.

It was thus not to be expected that the admixture of the three hereinbefore-described individual components in the ratios according to the invention would yield an oil with excellent properties for the purposes specified.

### EXAMPLE 1

A mixture was prepared from the following components:

- 63 percent by weight hexane-1,6-diol-3,5,5-trimethylhexanoate-2-ethylhexanoate
- 22 percent by weight 2,2-dimethylpropane-1,3-diol-pelargonate-3,5,5-trimethylhexanoate
- 15 percent by weight n-Oxo-octyl-n-Oxo-nonyl-2,2,4-trimethyladipate.

The properties of this admixture are listed in the table. As is seen from these data, this composition corresponds to the MIL-L-007808 F specification.

The alcohol components of the esters according to the invention are derived from alcohols obtained by Oxo-synthesis and hydrogenation of the hydroformylation products. The expression "n-Oxo" designates alcohols derived from alcohol mixtures obtained by hydroformylation of n-olefins (Oxo-synthesis) followed by hydrogenation of the hereby-obtained aldehydes. This Oxo synthesis is per se well known.

The ester n-Oxo-octyl-n-Oxo-nonyl-trimethyladipate has been hitherto not yet described. It is generally prepared in the manner described in Example 2.

### EXAMPLE 2

A 10-liter round-bottom flask was charged with 2,356 g of trimethyladipic acid, 1,720 g of n-Oxo-octanol and 1,880 g of n-Oxo-nonyanol. To said mixture were added 500 cm<sup>3</sup> of cumene as entrainer, and 3 g of paratoluene-sulfonic acid as catalyst. The solution was heated for more than 5 hours with stirring under reflux, with the temperature maintained at 155°C. During this time the theoretically formed amount of reaction water of 432 ml was carried out with the entrainer and separated with the aid of a laterally arranged water separator. Cumene was separated from the reaction product by distillation under the vacuum of a water-jet pump. Unreacted and only partially reacted components were separated from the cumene-free reaction product in two fractions by vacuum distillation. A first fraction of 370 g, comprising the acid containing components, distilled over in a temperature range between 50 and 140°C at 0.1 torr. A second fraction of 395 g was obtained in a temperature range between 110° and 154°C at 0.002 torr. The distillation residue of 4,660 g represented the desired crude ester oil. Thus, the yield amounted to 91 percent. The neutralization number of the ester was about 0.1 mg KOH per g, the ester number was about 264 mg KOH per g. The crude ester product was distilled, under a vacuum of 0.001 torr, to a residue of 90 g whereby the pure ester was obtained as a water-white product, which showed the following physical characteristics:

|                                       |       |       |
|---------------------------------------|-------|-------|
| Sp. Gr. d <sub>40</sub> <sup>20</sup> | =     | 0.918 |
| Viscosity in cSt                      |       |       |
| at 98.9°C                             | 3.21  |       |
| 37.8°C                                | 12.5  |       |
| -40 °C                                | 2110  |       |
| -53.9°C                               | 17100 |       |
| Viscosity-                            |       |       |
| Index                                 |       |       |
| Setting point °C                      | 139   |       |
| Flame point °C                        | -69   |       |
|                                       | 229   |       |

TABLE

| Test                                                                   | Standard value<br>(7808 Standards) | Determined<br>value<br>(Example 1) |
|------------------------------------------------------------------------|------------------------------------|------------------------------------|
| Viscosity (DIN 51 662):                                                |                                    |                                    |
| At 98.9° C.                                                            | At least 3.0 cSt.                  | 3.44 cSt.                          |
| At 37.8° C.                                                            | At least 11.0 cSt.                 | 13.49 cSt.                         |
| At -53.9° C.                                                           | Max. 13,000 cSt.                   | 12,489 cSt.                        |
| After further 3 hrs. at -53.9° C.                                      | Max. +6%                           | 12,414 cSt.                        |
| Flame point (ASTM D) at 760 torr.                                      | At least 204° C.                   | 223° C.                            |
| Flow point (ASTM D 97)                                                 | Below -60° C.                      | Below -67° C.                      |
| Evaporation loss (ASTM D 972) (6½ hrs., 204° C.)                       | Max. 35%                           | 30.6% by wt.                       |
| Corrosion- and oxidation-stability (FTM 791a-5308) (72 hrs., 175° C.): |                                    |                                    |
| Steel                                                                  | ±0.2 mg./cm. <sup>2</sup>          | +0.04 mg./cm. <sup>2</sup>         |
| Silver                                                                 | ±0.2 mg./cm. <sup>2</sup>          | +0.07 mg./cm. <sup>2</sup>         |
| Copper                                                                 | ±0.4 mg./cm. <sup>2</sup>          | +0.06 mg./cm. <sup>2</sup>         |
| MgAl 6                                                                 | ±0.2 mg./cm. <sup>2</sup>          | +0.05 mg./cm. <sup>2</sup>         |
| Al CuMg 2                                                              | ±0.2 mg./cm. <sup>2</sup>          | +0.03 mg./cm. <sup>2</sup>         |
| Viscosity at 37.8° C. after aging (72 hrs., 175° C.)                   | -5% to 15%                         | Below 1%.                          |
| Total acid number after aging (ASTM D 664) (72 hrs., 175° C.)          | Max. 2.3 mg. KOH/g.                | 0.24 mg. KOH/g.                    |
| Lead-corrosion (FTM 791a-5321) (1hr., 163° C.)                         | Max 6 mg./in. <sup>2</sup>         | -1.27 mg./in. <sup>2</sup>         |
| Silver-corrosion (FTM 791a-5305) (50 hrs., 232° C.)                    | 3.0 mg./in. <sup>2</sup>           | 0.3 mg./in. <sup>2</sup>           |
| Copper-corrosion (FTM 791a-5305) (50 hrs., 232° C.)                    | 3.0 mg./in. <sup>2</sup>           | 2.8 mg./in. <sup>2</sup>           |

25

30

35

40

45

50

55

60

65

70

What is claimed is:

1. Lubricant or power transmission fluid comprising 55 to 70 percent by weight hexane-1,6-diol-isononanoate-ethylhexanoate, 15 to 30 percent by weight 2,2-dimethylpropanediol-perlargonate-3,5,5 trimethylhexanoate and 10 to 20 percent by weight octyl-nonyl-trimethyladipate.

10 2. Lubricant or power transmission fluid, as claimed in claim 1, comprising 60 to 65 percent by weight hexane-1,6-diol-isononanoate-ethylhexanoate, 20 to 24 percent by weight 2,2-dimethylpropanediol-perlargonate-3,5,5 trimethylhexanoate and 13 to 17 percent by weight octyl-nonyl-trimethyladipate.

15 3. Lubricant or power transmission fluid, as claimed in claim 1, wherein said hexane-1,6-diol ester has an acid moiety mole ratio of about 0.9 to 1.1; said 2,2-dimethylpropanediol ester has an acid moiety mole ratio of about 0.9 to 1.1; and said trimethyladipate ester has an alcohol moiety mole ratio of about 0.9 to 1.1.

\* \* \* \* \*

25

75

UNITED STATES PATENT OFFICE  
CERTIFICATE OF CORRECTION

Patent No. 3,674,692 Dated July 4, 1972

Inventor(s) Herbert Gothel et al

It is certified that error appears in the above-identified patent and that said Letters Patent are hereby corrected as shown below:

Col. 2, line 39

"2,356" should be -- 2,256 --.

Col. 3, TABLE

At -53.9°C the determined value is "12,489," but it  
should be -- 12498. --.

Col. 3, TABLE

"Flame Point (ASTMD)" should be -- Flame Point (ASTMD 92)--.

Signed and sealed this 9th day of January 1973.

(SEAL)

Attest:

EDWARD M.FLETCHER,JR.  
Attesting Officer

ROBERT GOTTSCHALK  
Commissioner of Patents